

## UNITED STATES PATENT OFFICE

2,214,564

COATED PAPER AND METHOD OF  
MAKING THE SAME

William J. Montgomery and Donald B. Bradner,  
Hamilton, Ohio, assignors to The Champion  
Paper and Fibre Company, Hamilton, Ohio, a  
corporation of Ohio

No Drawing. Application January 26, 1938,  
Serial No. 187,074

9 Claims. (Cl. 91—68)

This invention relates to coated paper for printing and lithographic purposes, and particularly to paper having a "cast" surface produced by the processes described in Patent No. 2,029,273, issued January 28, 1936 to the present applicants, and in Patent No. 1,719,166, issued July 2, 1929 to Donald B. Bradner, one of the present applicants. It also relates to processes of producing said paper.

10 The paper of the present invention is eminently adapted to the production of can and bottle labels, of cigarette and other packages, for fancy candy box wrappings, for carton liners, for book jackets, magazine covers, advertising folders and other uses.

15 The most highly finished grades of supercalendered and brush-finished coated papers have insufficient gloss for present-day demands, as is evidenced by the extensive employment of varnish and lacquer, and the general use of Cellophane, either alone or pasted over printed paper.

20 The above designated Patent No. 1,719,166 describes the new cast coating process as it is practiced in applying to paper stock typical mineral 25 coating compositions such as have been employed for many years for making coated paper. The application of such coatings by the so-called "Bradner" process produces a coating of outstanding smoothness and gloss; a coating greatly 30 superior in these characteristics to coatings of similar composition when applied by any previously known method. Contrary, however, to what would be expected, these high gloss, exceptionally smooth "cast" coatings of the for- 35 mulae given in the Bradner patent are not as suitable for printing with gloss ink as coatings of the same composition when applied and supercalendered by the usual methods. The cast coatings are more absorbent to printer's ink than the 40 "supercalendered" coatings. In general, the ink after drying has a smooth velvety appearance with little gloss. This is an effect much sought after for many purposes, but it is a distinct disadvantage when a gloss ink effect is desired be- 45 cause the mirror finish is destroyed wherever it has been touched with ink, the dullness of the ink being accentuated by the greater gloss of the unprinted areas.

50 The primary object of the present invention is to provide a low cost mass production paper which when printed with suitable ink will have a brilliant gloss on both printed and unprinted portions without any subsequent varnishing or other operation.

55 In carrying out the present invention one of

the procedures described in the aforementioned Bradner patent or the Bradner and Montgomery patent may be employed. That is, the coating composition may be continuously applied to a traveling web of paper and subsequently dried or hardened in contact with a non-adhering finishing surface such as for instance a mirror-polished chromium plated drum or belt, or the coating may be applied to the polished surface and transferred to the traveling web. The present invention relates to the nature of the cast coated surface on the paper. The cast surface coating on our new paper ordinarily comprises a mixture of adhesive and filler, and is characterized by what the coated paper industry would consider an undesirable excess of adhesive.

For example, two samples of coated paper made with cast surface in accordance with the procedure described in the Bradner patent and substantially identical except for the proportions of filler (clay) and adhesive (casein) in the coating were tested on the Bausch and Lomb gloss meter in comparison with two similar samples having, respectively, the same coating compositions, but made according to the usual methods and supercalendered in accordance with the usual procedure of the art to obtain a high gloss. The results were as follows:

|                          | Cast finish  |    | Super-calendered finish |    |
|--------------------------|--------------|----|-------------------------|----|
|                          | A            | B  | A'                      | B' |
| Clay in coating.....     | parts.....   | 83 | 30                      | 83 |
| Casein in coating.....   | do.....      | 17 | 70                      | 17 |
| Bausch & Lomb gloss..... | percent..... | 76 | 94                      | 65 |
|                          |              |    |                         | 54 |

Viewed at low angle illumination under the microscope the surface of sample B was somewhat smoother than sample A, which in turn was definitely smoother than sample A', whilst sample B' was noticeably rougher than A'. Sample B printed in gloss ink presented on drying a gloss substantially equal to the gloss of the paper, indicating very little absorption of the ink by the paper, and the difference in ink absorption between samples A and B was much greater than between A' and B'.

The ratio of adhesive to filler required for the present purpose varies with the character of the filler employed. It is well recognized in the manufacture of "coated paper," that is, paper carrying supercalendered coatings of the composition designated as "mineral coatings" in

the Bradner patent, that different fillers require different amounts of adhesive to withstand "picking" on the printing press. In general, the finer the particle size the more adhesive is required. Thus ground limestone, a relatively coarse pigment, may be made into a sufficiently adherent coating with as little as 7 or 8% of casein, whereas finely precipitated calcium carbonate may require as much as 30% casein and satin white a still greater amount. It is also recognized that for a given filler the higher the adhesive content the more difficult it becomes to smooth out the coating in the supercalenders.

The one property which determines the printing quality of coated paper above everything else is its degree of smoothness. In making the best grades of supercalendered coated paper only enough adhesive is used to assure absence of "picking" or lifting on the press, for the reason that excess adhesive in the coating, other conditions being the same, impairs the gloss and smoothness imparted by the calendering. With the Bradner process the use of excess adhesive has the opposite effect. It enhances the gloss obtainable and improves the smoothness. The decreased absorbency makes it possible, by the use of gloss inks, to secure a gloss on the printing ink commensurate with the gloss on the paper itself. The decreased absorbency also reduces finger-marking which is otherwise especially disfiguring in the case of brightly colored high-gloss magazine covers, box covers, labels, etc., for which cast surface paper is a particularly attractive material.

By the expression "excess adhesive" we mean an excess over what would be commonly employed by an experienced paper-maker to insure the adhesion of the coating to the paper. This insurance involves a factor of safety over what might be the absolute minimum as would be determined by laboratory tests. Different batches of clay and other fillers supposedly of the same composition vary from one another in the amount of adhesive required to prevent "picking" of the coating in the printing operation. It is common practice, therefore, in making up the formulae for coating compositions to designate the amount of adhesive which experience has indicated will insure a proper adhesion of the coating to the paper stock, with any lot of designated filler and under any printing conditions.

Although a comparatively small excess of adhesive decreases the ink absorption of the cast coating, enhances its gloss and improves its smoothness, it is possible to increase the proportion of adhesive and decrease that of filler to any degree required to yield the results desired in any particular case. To secure opacity in coatings containing 30 per cent or more of adhesive it may be necessary to use in the filler a pigment of high refractive index such as zinc oxide, zinc sulphide, lithopone, or titanium oxide. For example, a coating composition of 40 per cent calcium carbonate, 10 per cent titanium oxide, and 50 per cent casein when cast upon the paper stock, produces a high-gloss opaque coating with low ink absorption.

In some cases a transparent coating is desirable, and in such cases if fillers having a refractive index nearly equal to that of the desired adhesive (such as clay and casein) are used, a coating may contain as much as 50 per cent or more of mineral filler and still be substantially transparent.

In the specific examples of coating composi-

tions employed in carrying out the present invention which we have given above, only casein is mentioned as the adhesive. Other adhesives known in the art may be used in lieu of casein with like results. For example, a coating composition consisting of 30 parts of blanc fixe, 30 parts of clay, and 40 parts of coating starch when cast on the surface of suitable paper stock in accordance with the process of the Bradner patent produces a finish of high gloss and smoothness and with a high resistance to penetration of oil-base printing inks.

Another adhesive that may be used is shellac. Due to the color in the shellac its use is largely confined to colored paper such as used for decorative wrappers or the like. For example, a coating composition consisting of 78% shellac, 4% sulphonated castor oil, and 18% dye in aqueous ammonia dispersion, when cast on a suitable paper stock produces a wrapping paper which is of exceptional gloss and smoothness and highly suitable for printing with gloss inks.

For colored coatings dyes, colored pigments, or mixtures of dyes and pigments may be employed. The above mentioned dyes, fillers, and pigments are ordinarily applied in aqueous dispersion. However, the present invention is not limited to the use of aqueous suspensions; organic solvents may be used; also thermoplastic gums or resins may be used, in which case the required cast surface is obtained by cooling in contact with the nonadhering finishing surface, and the solvent or suspending liquid may be dispensed with entirely. Ammonium stearate in the quantity specified in the above mentioned Montgomery and Bradner patent may be used with advantage in the examples given above to facilitate the casting operation.

In the foregoing specification we have referred to the coatings produced by the Bradner process as presenting a gloss finish. The paper embodying the invention of the present application is not, however, limited to paper presenting a gloss-finish. Either the gloss-finish or the matte finish of the Bradner process may be employed for the paper of the present application. Matte-finish paper is frequently used for printing with gloss inks, pleasing artistic effects and contrasts being thereby secured. Also the paper of the present invention possesses superior printing qualities in the matter of definition, uniformity, etc., and presents an enhanced smoothness over paper coated with the customary mineral coatings of the art such as referred to in the Bradner patent.

It is also to be understood that the specific formulae given above are intended to be by way of examples and not as limitations, and that the term filler is used in the appended claims to include mineral fillers, pigments, dyes, and other substances incorporated in paper coating compositions.

The expression "cast surfaced coating" is used in the appended claims to designate a coating which has been set from a plastic condition in contact with a solid, nonadhering casting surface described in the patents to Bradner, No. 1,719,166, or to Montgomery and Bradner, No. 2,029,273, so that the surface of the coating has substantially the same finish as the casting surface itself.

We claim:

1. Printing paper carrying a cast surface coating which comprises a major portion of adhesive and a minor portion of filler.

2. The process of manufacturing coated printing paper which comprises applying to paper a coating composition comprising filler and adhesive, said adhesive being present in an amount greater than 30% by weight of the coating composition calculated on a dry basis and imparting to the surface of the coating material a high degree of smoothness by causing the coating to harden in contact with a smooth, non-adhering 10 surface.

3. Process of manufacturing coated printing paper which comprises applying to paper a coating composition comprising filler and adhesive, said adhesive being present in an amount greater than 30% by weight of the coating composition calculated on a dry basis, contacting the coated 15 paper with a non-adhering finishing surface while the coating is in a plastic condition and rendering the coating non-plastic while in contact with said finishing surface.

4. The process of claim 2 in which the coating composition comprises a mineral filler and an adhesive.

5. Printing paper carrying a cast surfaced

coating which contains an adhesive in amount more than 30% by weight of the total coating calculated on the dry basis.

6. Printing paper carrying a cast surfaced coating which contains as essential ingredients 5 adhesive and mineral filler, the mineral filler being in amount less than 70% by weight of the total coating calculated on the dry basis.

7. The paper of claim 6 in which the adhesive used is casein.

8. The paper of claim 6 in which the mineral filler is of high refractive index as compared with the refractive index of the adhesive.

9. Process of making cast surfaced coated paper which comprises applying to paper a coating composition comprising an aqueous dispersion containing shellac, the shellac comprising more than 30% by weight of the total coating calculated on the dry basis, and imparting to the surface of the coating material a high degree of 15 smoothness by drying the coating in contact with a smooth, nonadhering surface.

WILLIAM J. MONTGOMERY.

DONALD B. BRADNER.